

## 1

3,113,864

REDUCING FOG IN REVERSAL COLOR FILMS  
PROCESSED IN DEVELOPERS CONTAINING  
COUPLERS

Barbara C. Yager, Catherine M. Spath, and Judith A. Schwan, Rochester, N.Y., assignors to Eastman Kodak Company, Rochester, N.Y., a corporation of New Jersey

No Drawing. Filed June 11, 1959, Ser. No. 819,539  
14 Claims. (Cl. 96—22)

This invention relates to color photography, and more particularly, to a method of processing multi-layer color films or papers in such a manner as to reduce color fog and give maximum color density.

In multi-layer photographic elements used for color photography, there are usually three selectively sensitive emulsion layers coated on one side of a single support. For example, the uppermost layer is generally blue-sensitive, the next layer is generally green-sensitive, while the emulsion layer adjacent the support is generally red-sensitive. Between the blue-sensitive and green-sensitive layers is a filter layer for absorbing blue radiation which may be transmitted through the blue-sensitive layer. The multi-layer coating can also have other interlayers for specialized purposes. Such multi-layer materials have been previously described in the prior art, such as Mannes et al. U.S. Patent 2,252,718, issued August 19, 1941. Other arrangements of the sensitive layers are also known.

Color materials of the type employed in the instant invention are those intended primarily for reversal processes, wherein the exposed material is given a conventional black-and-white development, followed by a reversal exposure, or exposures, and color development.

Our invention is particularly useful in processing reversal color materials, wherein the color-forming components or couplers are incorporated in the color developers.

It is, therefore, an object of our invention to provide an improved method of inhibiting color fog and increasing the maximum color density of reversal color materials intended for processing in color developers containing color-forming materials or couplers. Another object is to provide a method of inhibiting color development fog in the various layers of multilayer color materials. Other objects will become apparent from a consideration of the following description and examples.

During the black-and-white development of multi-layer color materials, fog centers are introduced into the unexposed regions, and upon selective reversal re-exposure and subsequent color development, these unexposed areas have deposited therein coupled color-forming materials, resulting in severe loss of color quality. This loss of color quality is particularly severe in the processing of red-sensitized photographic silver halide emulsions, which are processed in a reversal color developer containing the coupling material, resulting in the development of cyan fog in the blue-and-green sensitive layers. This fog is particularly severe in emulsions which contain any of the known chemical sensitizing agents, such as gold sensitizers, sulfur sensitizers, etc., or polyethylene-glycol type sensitizers.

We have discovered a new method for eliminating or substantially reducing the formation of color fog in the unexposed layers of multilayer color materials intended for reversal processing in a color developer containing the color-forming materials or couplers. This method consists in contacting the multilayer color material after negative development in the black-and-white developer, but before color development, with an aqueous solution containing certain benzothiazolium or naphthothiazolium salts. This treatment allows normal color development to take place in the exposed layer, but inhibits the development of undesired fog in the unexposed layers.

## 2

Of course, the reversal process used in the present invention is one which has been previously described in the prior art, and it is to be understood that our invention resides in a modification of this prior art technique.

That is, it is known that in reversal processing, a colored image can be formed by adding to certain color developing solutions, a compound which couples during development with the oxidation product of the developing agent, thus forming a colored compound which is deposited adjacent to the developed silver halide grains or the silver image, during such color development. The color density improving treatment employed in our invention is applied to the multilayer color material after conventional negative development in a black-and-white developer, and before or after one of the reversal re-exposures for the differentially sensitized emulsion layers. The multilayer color material is, of course, given successive color development treatments for each of the differentially sensitized emulsion layers after reversal reexposure for each emulsion layer. The compounds employed in conjunction with the color developing agents and which couple with the oxidation products of the developing agents during development are generally referred to as color-forming compounds, or couplers. Such compounds usually belong to one of three widely known types, i.e., pyrazolone couplers, phenol couplers, and open-chain ketomethylene couplers. These couplers produce, respectively, magenta, cyan and yellow images.

The quaternary salts useful in practicing our invention comprise compounds represented by the following general formula:

(I)



wherein R represents a hydrogen atom or a lower alkyl group, such as methyl, ethyl, etc. (e.g., an alkyl group containing from 1-2 carbon atoms), R<sub>1</sub> represents a hydrogen atom, an aryl group (e.g., phenyl, o-, m- and p-tolyl, o-, m- and p-methoxyphenyl, etc.), or an arylene-thiazolyl group (e.g., 2-benzothiazolyl, 3-benzothiazolyl, 2-(β-naphthothiazolyl) etc.) D represents the non-metallic atoms necessary to complete an aromatic nucleus (e.g., benzene, naphthalene, etc., as well as their substitution products, including such members substituted by methyl, ethyl, methoxyl, ethoxyl, etc.), n represents a positive integer of from 1-26 (provided that n represents a positive integer of only from about 1-3 when R<sub>1</sub> represents an aryl group) and X represents an acid radical, such as perchlorate, bromide, benzenesulfonate, toluenesulfonate, methyl sulfate, ethyl sulfate, etc.

45 A particularly useful group of quaternary salts embraced by Formula I above includes the compounds represented by the following general formula:

50

55

(II)



wherein R, D and X each have the values given above, and m represents a positive integer of from about 1-26.

Typical quaternary salts embraced by Formula I above include the following:

(1)



Decamethylene-bis-benzothiazolium perchlorate

(2)



3-ethylbenzothiazolium-p-toluenesulfonate

(3)



3-hexylbenzothiazolium-p-toluenesulfonate

(3a)



(4)



3-nonylbenzothiazolium-p-toluenesulfonate

(5)



Trimethylene-bis-2-methylbenzothiazolium bromide

(6)



Decamethylene-bis(2-methylbenzothiazolium) perchlorate

(7)



3-(2-benzothiazolylmethyl)-2-methylbenzothiazolium-p-toluenesulfonate

(8)



2-methyl-β-naphthothiazolium metho-p-toluenesulfonate

(9)



Ethylene-bis-benzothiazolium bromide

(10)



Pentamethylene-bis-benzothiazolium perchlorate

(11)



Hexamethylene-bis-benzothiazolium perchlorate

(11a)



3-benzylbenzothiazolium chloride

(12)



Heptamethylene-bis-benzothiazolium perchlorate

(13)



Nonamethylene-bis-benzothiazolium perchlorate

(14)



Hexacosane-1,26-bis-benzothiazolium perchlorate

Many of these quaternary compounds have been previously described in the prior art. For example, the bis compounds represented by Formula II can be prepared according to the methods described in Wilson U.S. Patent 2,425,774, issued August 19, 1947, as well as by the method described by Allen and Wilson U.S. Patent 2,694,716, issued November 16, 1954. Such methods generally comprise the fusion of a heterocyclic base with an alkylene halide. Such techniques are well known to those skilled in the art. Alkyl esters of organic sulfonic acids can also be fused with thiazole bases to provide the salts of our invention.

75 The cycloammonium salts useful in practicing our in-

vention are employed in the form of their aqueous solutions. The amount of quaternary salt used in the solutions can be varied, depending upon the particular emulsions employed, the concentration of silver halides in the emulsions, etc. In general, we have found that concentrations of from about 0.25 to 1.0 gram per liter of solution are particularly effective. However, the most advantageous concentration for a particular color material can be determined by running a series of test strips of silver halide emulsions through a reversal color process of the type described herein, the concentration of the quaternary salt in the treating solution being varied. The multilayer color materials treated in our invention can be immersed in the treating solution, or for continuous processes, the treating solution may be applied, for example, by means of rollers, etc. In general, it has been found desirable to give the multilayer color material a short washing treatment after treatment with the quaternary salt in order to avoid spotting.

The treatment of the multilayer color materials of our invention can be made either before or after the reversal re-exposure step. However, it must be made after the negative development in the black-and-white developer, but before development in the color developer. We have found that the beneficial effects of the quaternary salts of our invention cannot be obtained if these materials are incorporated in the emulsions. In some instances, the thiazolium salt (e.g., Compound 11a) can be incorporated in the color developing solution where it is soluble in such solution.

The advantages of our invention have been obtained in a large number of multilayer color materials and the effect is not dependent upon any particular emulsions or developing compositions. The effects have been found to be outstanding when the red-sensitive layer is color developed first in that the development fog centers present in the blue and green layers, which were not re-exposed after black-and-white development, do not develop spontaneously to form unwanted cyan dye and the resultant loss of color quality in these layers. However, the effects are apparent, though not as outstanding when the photographic silver halide emulsion layers intended for the production of magenta or yellow images are color developed first. Typical couplers for use in the color developers of our invention comprise the following:

#### COUPLERS FOR USE IN COLOR DEVELOPERS

##### Cyan Couplers

- (1) 5-benzenesulfonamino-1-naphthol
- (2) 2,4-dichloro-5-benzenesulfonamino-1-naphthol
- (3) 2,4-dichloro-5-(p-toluenesulfonamino)-1-naphthol
- (4) 5-(1,2,3,4-tetrahydronaphthalene-6-sulfonamino)-1-naphthol
- (5) 2,4-dichloro-5-(4'-bromodiphenyl-4-sulfonamino)-1-naphthol
- (6) o-( $\beta$ -Naphthalenesulfonamino)-1-naphthol
- (7) 5-(m-nitrobenzenesulfonamino)-1-naphthol
- (8) 5-(quinoline-5-sulfonamino)-1-naphthol (U.S. 2,362,598)
- (9) 2-acetylaminio-5-methylphenol
- (10) 2-benzoylamino-3,5-dimethylphenol
- (11) 2- $\alpha$ -(p-tert. amylphenoxy)-n-butyrylaminio-5-methylphenol
- (12) 2- $\alpha$ -(p-tert. amylphenoxy)-n-butyrylaminio-4-chloro-5-methylphenol
- (13) 2-(p-tert. amylphenoxy-p-benzoyl)amino-4-chloro-5-methylphenol
- (14) 2-(4'-tert. amyl-3'-phenoxybenzoylaminio)-3,5-dimethyl-1-phenol
- (15) 2-phenylacetylaminio-4-chloro-5-methylphenol
- (16) 2-benzoylamino-4-chloro-5-methylphenol
- (17) 2-aminoacetylaminio-4-chloro-5-methylphenol
- (18) 2-{4'-[ $\alpha$ -(4'-tert. amylphenoxy)-n-butyrylaminio]-benzoylaminio}-4-chloro-5-methylphenol

- (19) 2-{4'-[3'-4'''-tert. amylphenoxy)-benzoylamino]-benzoylaminio}-4-chloro-5-methylphenol
- (20) 2-p-nitrobenzoylaminio-4-chloro-5-methylphenol
- (21) 2-m-aminobenzoyl-4-chloro-5-methylphenol
- (22) 2-acetamino-4-chloro-5-methylphenol
- (23) 2-(4'-sec. amylbenzamido)-4-chloro-5-methylphenol
- (24) 2-(4'-n-amyloxybenzamino)-4-chloro-5-methylphenol

##### Magenta Couplers

- (25) 1-phenyl-3-acetylaminio-5-pyrazolone
- (26) 1-phenyl-3-propionylaminio-5-pyrazolone
- (27) 1-phenyl-3-dichloroacetylaminio-5-pyrazolone
- (28) 1-phenyl-3-benzoylaminio-5-pyrazolone
- (29) 1-phenyl-3-(m-aminobenzoyl)-amino-5-pyrazolone
- 15 hydrochloride
- (30) 1-phenyl-3-(diamylbenzoyl)amino-5-pyrazolone
- (31) 1-phenyl-3-phenylcarbamylaminio-5-pyrazolone
- (32) 1-phenyl-3-phenoxyacetylaminio-5-pyrazolone
- (33) 1-phenyl-3-p-aminobenzoylaminio-5-pyrazolone
- 20 (34) 1-phenyl-3-(o-carboxybenzoyl)amino-5-pyrazolone
- (35) 1-phenyl-3-palmitylaminio-5-pyrazolone
- (36) 1-phenyl-3-(p-sec. amylbenzenesulfonylaminio)-5-pyrazolone
- (37) 1-phenyl-3-[p-(p-sec. amylbenzoyl)aminobenzoyl-amino]-5-pyrazolone
- 25 (38) 1-m-tolyl-3-[m-( $\beta$ -phenylpropionyl)aminobenzoyl-amino]-5-pyrazolone
- (39) 1-m-tolyl-3-(2,4-di-tert. butyl-m-tolyloxyacetyl-amino)-5-pyrazolone
- 30 (40) 1-[p-(p'-tert. butylphenoxy)phenyl]-3-[p-(benzoyl-amino)-benzoylaminio]-5-pyrazolone
- (41) 1-(p-tert. butylphenoxyphenyl)-3-(p-n-amyloxy-benzoylaminio)-5-pyrazolone
- 35 (42) 1-[p-(p'-tert. butylphenoxy)phenyl]-3-(3,5-di-methoxybenzoyl)amino-5-pyrazolone
- (43) 1-[p-(p'-tert. butylphenoxy)phenyl]-3-[m-(p-toluenesulfonylaminio)benzoylaminio]-5-pyrazolone
- (44) 1-[p-(3,5-dimethylphenoxy)phenyl]-3-(4-n-amyloxy-3-methylbenzoylaminio)-5-pyrazolone
- 40 (45) 3-(p-nitrophenoxyacetylaminio)-1-(2,4,6-trichlorophenyl)-5-pyrazolone

##### Yellow Couplers

- (46) p-( $\omega$ -Benzoylacetamino)benzenesulfonamide
- 45 (47) p-( $\omega$ -Benzoylacetamino)benzenesulfon-N-methylamide
- (48) p-( $\omega$ -Benzoylacetamino)benzenesulfonanilide
- (49) 4-benzenesulfonamino- $\omega$ -benzoylacetanilide
- (50) 4-(p-toluenesulfonamino)- $\omega$ -benzoylacetanilide
- 50 (51) 4-(p-laurylbenzenesulfonamino)- $\omega$ -benzoylacetanilide
- (52) 1,4-di-[p-(benzoylacetamino)benzenesulfonamino]-benzene
- (53) N,N-di-(p-benzoylacetaminophenyl)benzene-1,3-disulfonamide
- 55 (54) N-(p-benzoylacetaminophenyl)-4-[p-(benzoylacetamino)-benzenesulfonamido]benzenesulfonamide
- (55) N4-benzoylacetyl-N'-(2-benzothiazolyl)sulfanilamide
- 60 (56) p-Acetoacetaminobenzenesulfon- $\beta$ -naphthalide
- (57) p-Furoylacetaminobenzenesulfon-N-cyclohexylamide
- (58) p-(4-ethoxybenzoylacetamino)benzenesulfonamide
- (59) Terephthaloyl-bis[(p-N-aminosulfonamide)acetanilide]
- 65 (60) p-Quinoline-8-sulfonamino)- $\omega$ -benzoylacetanilide
- (61) p-Acetoacetamino-o-methylbenzenesulfon-N-anilide
- (62) N,N'-di-(p-benzoylacetaminophenol)naphthalene-1,5-disulfonamide
- 70 (63) p-(Benzenesulfonamino)benzoylacetone
- (64) N-benzoylacet-o-anisidine

The color-forming developers useful in our invention have been previously described in the prior art, and our invention is not to be restricted to the use of any particular color-forming developer. Particularly useful

color-forming developers comprise those containing primary aromatic amines, containing an amino (substituted or not) or hydroxyl substituent. Phenylenediamines and substituted derivatives thereof containing a primary amino group have been found to provide particularly useful results. Typical of such color-forming developers are the sulfonamido substituted p-phenylenediamines disclosed in Weissberger U.S. Patent 2,548,574, issued April 10, 1951, the substituted p-phenylenediamines disclosed in Weissberger et al. U.S. Patent 2,566,271, issued August 28, 1951. Of course, other phenylenediamine color-forming developers can be employed with equal facility in the process of our invention.

The first, or negative, developer employed in the process of our invention is generally a rapid developer of the "MQ" type, i.e., a combination of hydroquinone and Elon (p-N-methylaminophenol) developer, although other high-speed developers, such as those containing Phenidone can also be employed.

The following examples will serve to illustrate more fully the manner of practicing our invention.

#### EXAMPLE 1

A portion of a red-sensitized, gelatino-silver-bromiodide emulsion which had been sensitized with a sulfur compound, a gold compound and a small amount of the oleyl ether of a polyethyleneglycol having a molecular weight of about 900 was coated on a cellulose acetate film support. The coating was then dried and exposed to a step table for  $\frac{1}{100}$  second, using a 500-watt, 3000° K. light source, filtered with a Wratten No. 29 Filter (i.e., a filter transmitting only light from about 610 to 700 millimicrons) and a 0.8 neutral density filter, on an Eastman Type Ib Sensitometer. The exposed coating was then developed for 10 minutes in a developer having the following composition:

|                                | Grams |
|--------------------------------|-------|
| Elon developing agent          | 2.0   |
| Sodium sulfite, desiccated     | 90.0  |
| Hydroquinone                   | 8.0   |
| Sodium carbonate, monohydrated | 52.5  |
| Potassium bromide              | 5.0   |
| Cold water to make 1.0 liter.  |       |

The coating was washed for 2 minutes with water.

The coating was then given a reversal re-exposure (15 seconds' flash) with a No. 2 Photoflood Filter with a Lowry red Filter No. 92, set at a distance of about one meter. The coating was developed to an adequate D-max. for 20 minutes in a developer having the following composition:

|                                  |    |      |
|----------------------------------|----|------|
| Sulfuric acid (conc.)            | cc | 1.5  |
| Sodium hexametaphosphate         | g  | 0.5  |
| Sodium sulfite (anhydrous)       | g  | 5.0  |
| Color developer <sup>1</sup>     | g  | 0.6  |
| Sodium carbonate (monohydrate)   | g  | 15.0 |
| Potassium bromide                | g  | 0.25 |
| Potassium iodide (0.1% solution) | cc | 2    |
| Coupler <sup>2</sup>             | g  | 1.2  |
| Sodium hydroxide                 | g  | 0.3  |
| Carbowax 1540                    | g  | 1.0  |
| Water to make one liter.         |    |      |

<sup>1</sup> 4-amino-3-methyl-N,N-diethylaniline hydrochloride.

<sup>2</sup> 2,4-dichloro-5-(p-toluenesulfonamido)-1-naphthol.

The coating was washed for 10 minutes in water and immersed for 2 minutes in a silver bleach bath having the following composition:

|                          |     |
|--------------------------|-----|
| Potassium ferricyanide   | 100 |
| Potassium bromide        | 10  |
| Borax                    | 7.5 |
| Boric acid               | 5.0 |
| Water to make one liter. |     |

The coating was then treated for 2 minutes in a fixing bath having the following composition:

|    |                                   |     |
|----|-----------------------------------|-----|
| G. | Sodium thiosulfate (pentahydrate) | 200 |
| 5  | Sodium sulfite (anhydrous)        | 10  |
|    | Water to make one liter.          |     |

The coating was then washed in water for 10 minutes and dried. In order to obtain a measure of the cyan fog, an identical strip of coating was put through the same process, except that the flash re-exposure was omitted.

Additional strips of the same coating were put through the same process except that the strips were treated for 2 minutes in an aqueous solution containing Compound 1 above, after red re-exposure, but before color development. After treatment in this pre-bath, the strips were washed for 2 minutes in water. The treating solution was obtained by dissolving 1.0 g. of Compound 1 in 175 cc. of methyl alcohol and diluting the solution to 1 liter with water. The D-max. and cyan fog for each of these coatings was measured, the following results being obtained:

| 25 | Compound No.     | Cyan D-Max. | Cyan Fog |
|----|------------------|-------------|----------|
|    | Control (none)   | 3.32        | 0.52     |
|    | 1 (1.0 g./liter) | 3.56        | 0.23     |

#### EXAMPLE 2

30 In a manner similar to that described above, a multilayer color material was processed both with and without the pre-bath treatment in an aqueous solution containing Compound 1 above (i.e., decamethylene-bis-benzothiazolium perchlorate). The multilayer color material comprised a conventional cellulose acetate film support having coated thereon in order, a gelatin layer, a red-sensitized silver halide emulsion layer, a green-sensitized silver halide emulsion, a yellow filter layer comprising Carey Lea silver, and a blue-sensitive silver halide emulsion layer. Each of the silver halide emulsion layers was gold and sulfur sensitized as in Example 1, and each contained a small amount of a polyethylene glycol sensitizer having a molecular weight of about 900.

35 Processing of the strips of coating was exactly as described in Example 1 above, except that the black-and-white development was for 12 minutes, instead of 10, and 0.50 gram of H-acid was added to the color developer. The following results were obtained:

| 50 | Compound No. | Relative Speed | Cyan D-Max. | Cyan Fog |
|----|--------------|----------------|-------------|----------|
|    | Control      | 100            | 3.70        | 1.05     |
|    | 1            | 101            | 3.23        | 0.26     |

55 The speeds were read at a density of 0.3 below maximum density.

#### EXAMPLE 3

60 A portion of a blue-sensitive, gelatino-silver-bromiodide emulsion which had been sensitized with a sulfur compound, a gold compound and a polyethyleneglycol sensitizer having a molecular weight of about 900 was coated onto a cellulose acetate support. The coating was then dried and cut into several strips. One strip of the coating was exposed to a step table for  $\frac{1}{100}$  second to a 500-watt, 3000° K. light source, filtered with a Wratten No. 49 Filter (i.e., a filter transmitting only light of wavelengths between about 400 and 510 millimicrons) on an Eastman Type Ib Sensitometer. The exposed strip

65 was developed for 10 minutes in a hydroquinone-Elon Developer of the type used in Example 1, and washed for 2 minutes in water.

70 The strip was given a reversal re-exposure for about 15 seconds (flash) with a No. 2 Photoflood set at a distance of about 1 meter. The strip was then developed

for 15 minutes in a color developer having the following composition:

|                                  |     |      |
|----------------------------------|-----|------|
| Sodium hexametaphosphate         | g.  | 0.5  |
| Sodium sulfide (des.)            | g.  | 5.0  |
| Color developer <sup>1</sup>     | g.  | 1.0  |
| Sodium carbonate (monohydrate)   | g.  | 20.0 |
| Sodium bromide                   | g.  | 0.25 |
| Potassium iodide (0.1% solution) | cc. | 2    |
| Coupler <sup>2</sup>             | g.  | 1.0  |
| Carbowax 1540                    | g.  | 1.0  |
| Sodium hydroxide                 | g.  | 0.50 |
| Water to make one liter.         |     |      |

<sup>1</sup> 2-amino-5-diethylaminobenzene hydrochloride.  
<sup>2</sup>  $\omega$ -Benzoyl-4-(*p*-toluenesulfonamido)acetanilide.

Carbowax 1540 is a polyethylene oxide resin.

The strip was then washed, bleached, fixed and washed exactly as described in Example 1 above. In order to determine fog, a duplicate strip was processed, except that the reversal re-exposure with the Photoflood was omitted.

In a manner described immediately above, duplicate strips were processed to a yellow image, except that the strips were bathed for 2 minutes in an aqueous solution containing decamethylene-bis-benzothiazolium perchlorate (1.0 g./liter), followed by a 2-minute wash after reversal re-exposure, but before color development. The results obtained were as follows:

| Compound No.                | Yellow D-Max. | Yellow Fog   |
|-----------------------------|---------------|--------------|
| Control<br>1 (1.0 g./liter) | 1.82<br>1.52  | 0.64<br>0.30 |

#### EXAMPLE 4

In exactly the manner described in Example 2 above (i.e., with 12 minutes' black-and-white development and with color developer containing 0.5 g. of H-acid), strips of the multilayer color material described in Example 2 were processed, both with and without treatment in one of the pre-baths containing a quaternary salt. The bromide emulsions were sulfur and gold sensitized and contained a polyethyleneglycol sensitizer as described in Example 2. The pre-baths contained 1.0 g./liter of quaternary salt. The cyan D-max. and cyan fog for the film strips are given below:

| Compound No.                                                                     | Cyan<br>D-Max. | Cyan<br>Fog |
|----------------------------------------------------------------------------------|----------------|-------------|
| Control—no treatment                                                             | 3.80           | 1.18        |
| Decamethylene bis benzothiazolium perchlorate                                    | 2.90           | .28         |
| 3-Ethyl benzothiazolium <i>p</i> -toluene sulfonate                              | 3.85           | .59         |
| 3-Hexyl benzothiazolium <i>p</i> -toluene sulfonate                              | 3.88           | .38         |
| 3-Nonyl benzothiazolium <i>p</i> -toluene sulfonate                              | 2.75           | .22         |
| 3,3'-Trimethylene bis-(2-methyl benzothiazolium) bromide                         | 2.84           | .28         |
| Decamethylene bis (2-methyl benzothiazolium) perchlorate                         | 3.12           | .32         |
| 3-(2-Benzothiazolyl methyl)-2-methyl benzothiazolium <i>p</i> -toluene sulfonate | 3.18           | .23         |
| 2-Methyl- $\beta$ -naphthothiazolium methyl <i>p</i> -toluene sulfonate          | 3.00           | .48         |
| Ethylene bis benzothiazolium bromide                                             | 3.55           | .48         |
| Pentamethylene bis benzothiazolium perchlorate                                   | 3.16           | .17         |
| Hexamethylene bis benzothiazolium perchlorate                                    | 3.20           | .24         |
| Heptamethylene bis benzothiazolium perchlorate                                   | 3.21           | .28         |
| Nonamethylene bis benzothiazolium perchlorate                                    | 3.23           | .32         |
| Hexacosane-1,26-bis-benzothiazolium perchlorate                                  | 3.20           | .46         |

As evident from the above data, our invention is concerned primarily with treatment of the ordinarily employed gelatin-silver-halide developing-out emulsions. While the examples are concerned primarily with silver bromide emulsions, it is to be understood that other silver halide emulsions can be employed, such as silver chloride, -chlorobromide, -chloroiodide, -chlorobromiodide and -bromide developing-out emulsions. These emulsions can be coated in the usual manner on any support, such as glass, cellulose nitrate film, cellulose acetate film, polyvinylacetyl resin film, etc.

The emulsions can be chemically sensitized by any of 75

the accepted procedures. The emulsions can be digested with naturally active gelatin, or sulfur compounds can be added such as those described in Sheppard U.S. Patent 1,574,944, issued March 2, 1926, Sheppard et al. U.S. Patent 1,623,499, issued April 5, 1927, and Sheppard et al. U.S. Patent 2,410,689, issued November 5, 1946.

The emulsions can also be treated with salts of the noble metals such as ruthenium, rhodium, palladium, iridium, and platinum. Representative compounds are ammonium chloropalladate, potassium chloroplatinate, and sodium chloropalladite, which are used for sensitizing in amounts below that which produces any substantial fog inhibition, as described in Smith and Trivelli U.S. Patent 2,448,060, issued August 31, 1948, and as antifog-gants in higher amounts, as described in Trivelli and Smith U.S. Patents 2,566,245, issued August 28, 1951, and 2,566,263, issued August 28, 1951.

The emulsions can also be chemically sensitized with gold salts as described in Waller et al. U.S. Patent 2,399,083, issued April 23, 1946, or stabilized with gold salts as described in Damschroder U.S. Patent 2,597,856, issued May 27, 1952, and Yutzy and Leermakers U.S. Patent 2,597,915, issued May 27, 1952. Suitable compounds are potassium chloroaurite, potassium aurithiocyanate, potassium chloroaurate, auric trichloride and 2-aurosulfo-benzothiazole methochloride.

The emulsions can also be chemically sensitized with reducing agents such as stannous salts (Carroll U.S. Patent 2,487,850, issued November 15, 1949), polyamines, such as diethyl triamine (Lowe and Jones U.S. Patent 2,518,698, issued August 15, 1950), polyamines, such as spermine (Lowe and Allen U.S. Patent 2,521,925, issued September 12, 1950), or bis( $\beta$ -aminoethyl) sulfide and its water-soluble salts (Lowe and Jones U.S. Patent 2,521,926, issued September 12, 1950).

The emulsions can also be optically sensitized with cyanine and merocyanine dyes, such as those described in Brooker U.S. Patents 1,846,301, issued February 23, 1932; 1,846,302, issued February 23, 1932; and 1,942,854, issued January 9, 1934; White U.S. Patent 1,990,507, issued February 12, 1935; Brooker and White U.S. Patents 2,112,140, issued March 22, 1938; 2,165,338, issued July 11, 1939; 2,493,747, issued January 10, 1950, and 2,739,964, issued March 27, 1956; Brooker and Keyes U.S. Patent 2,493,748, issued January 10, 1950; Sprague U.S. Patents 2,503,776, issued April 11, 1950, and 2,519,001, issued August 15, 1950; Heseltine and Brooker U.S. Patent 2,666,761, issued January 19, 1954; Heseltine U.S. Patent 2,734,900, issued February 14, 1956; Van Lare U.S. Patent 2,739,149, issued March 20, 1956; and Kodak Limited British Patent 450,958, accepted July 15, 1936.

The emulsions can also be stabilized with the mercury compounds of Allen, Byers and Murray U.S. Patent 2,728,663, issued December 27, 1955; Carroll and Murray U.S. Patent 2,728,664, issued December 27, 1955; and Leubner and Murray U.S. Patent 2,728,665, issued December 27, 1955; the triazoles of Heimbach and Kelly U.S. Patent 2,444,608, issued July 6, 1948; the azaindenes of Heimbach and Kelly U.S. Patents 2,444,605 and 2,444,606, issued July 6, 1948; Heimbach U.S. Patents 2,444,607, issued July 6, 1948, and 2,450,397, issued September 28, 1948; Heimbach and Clark U.S. Patent 2,444,609, issued July 6, 1958; Allen and Reynolds U.S. Patents 2,713,541, issued July 19, 1955, and 2,743,181, issued April 24, 1956; Carroll and Beach U.S. Patent 2,716,062, issued August 23, 1955; Allen and Beifuss U.S. Patent 2,735,769, issued February 21, 1956; Reynolds and Sagal U.S. Patent 2,756,147, issued July 24, 1956; Allen and Sagura U.S. Patent 2,772,164, issued November 27, 1956, and those disclosed by Birr in "Z. wiss. Phot.", vol. 47, 1952, pages 2-28; the disulfides of Kodak Belgian Patent 569,317, issued July 31, 1958; the quaternary benzothiazolium compounds of Brooker and Staud U.S. Patent 2,131,038, issued September 27, 1938, or the polymethylene bis-benzothiazolium salts of Allen and Wilson U.S. Patent

2,694,716, issued November 16, 1954; or the zinc and cadmium salts of Jones U.S. Patent 2,839,405, issued June 17, 1958.

The emulsions may also contain speed-increasing compounds of the quaternary ammonium type of Carroll U.S. Patent 2,271,623, issued February 3, 1942; Carroll and Allen U.S. Patent 2,288,226, issued June 30, 1942; and Carroll and Spence U.S. Patent 2,334,864, issued November 23, 1943; and the polyethyleneglycol type of Carroll and Beach U.S. Patent 2,708,162, issued May 10, 1955.

The emulsions may contain a suitable gelatin plasticizer such as glycerin; a dihydroxy alkane such as 1,5-pentane diol as described in Milton and Murry U.S. application Serial No. 588,951, filed June 4, 1956; an ester of an ethylene bis-glycolic acid such as ethylene bis(methyl glycolate) as described in Milton U.S. application Serial No. 662,564, filed May 31, 1957; bis-(ethoxy diethylene glycol) succinate as described in Gray U.S. application Serial No. 604,333, filed August 16, 1956, or a polymeric hydrosol as results from the emulsion polymerization of a mixture of an amide of an acid of the acrylic acid series, and acrylic acid ester and a styrene-type compound as described in Tong U.S. Patent 2,852,386, issued September 16, 1958. The plasticizer may be added to the emulsion before or after the addition of a sensitizing dye, if used.

The emulsions may be hardened with any suitable hardener for gelatin such as formaldehyde; a halogen-substituted aliphatic acid such as mucobromic acid as described in White U.S. Patent 2,080,019, issued May 11, 1937; a compound having a plurality of acid anhydride groups such as 7,8-diphenylbicyclo (2,2,2)-7-octene-2,3,5,6-tetra-carboxylic dianhydride, or a dicarboxylic or a disulfonic acid chloride such as terephthaloyl chloride or naphthalene-1,5-disulfonyl chloride as described in Allen and Carroll U.S. Patents 2,725,294, and 2,725,295, both issued November 29, 1955; a cyclic 1,2-diketone such as cyclopentane-1,2-dione as described in Allen and Byers U.S. Patent 2,725,305, issued November 29, 1955; a bisester of methane-sulfonic acid such as 1,2-di-(methane-sulfonyloxy)-ethane as described in Allen and Laakso U.S. Patent 2,726,162, issued December 6, 1955; 1,3-dihydroxymethylbenzimidazol-2-one as described in July, Knott and Pol-lak U.S. Patent 2,732,316, issued January 24, 1956; a dialdehyde or a sodium bisulfite derivative thereof, the aldehyde groups of which are separated by 2-3 carbon atoms, such as  $\beta$ -methyl glutaraldehyde bis-sodium bisulfite as described in Allen and Burness U.S. Patent application Serial No. 556,031, filed December 29, 1955; a bis-aziridine carboxamide such as trimethylene bis(1-aziridine carboxamide) as described in Allen and Webster U.S. Patent application Serial No. 599,891, filed July 25, 1956; or 2,3-dihydroxy dioxane as described in Jeffreys U.S. Patent 2,870,013, issued January 20, 1959.

The emulsions may contain a coating aid such as saponin; a lauryl or oleyl monoester of polyethyleneglycol as described in Knox and Davis U.S. Patent 2,831,766, issued April 22, 1958; a salt of a sulfated and alkylated polyethyleneglycol ether as described in Knox and Davis U.S. Patent 2,719,087, issued September 27, 1955; an acylated alkyl taurine such as the sodium salt of N-oleoyl-N-methyl taurine as described in Knox, Twardokus and Davis U.S. Patent 2,739,891, issued March 27, 1956; the reaction product of a dianhydride of tetracarboxybutane with an alcohol or an aliphatic amine containing from 8 to 18 carbon atoms which is treated with a base, for example, the sodium salt of the monoester of tetracarboxybutane as described in Knox, Stenberg and Wilson U.S. Patent 2,843,487, issued July 15, 1958; a water-soluble maleopimarate or a mixture of a water-soluble maleopimarate and a substituted glutamate salt as described in Knox and Fowler U.S. Patent 2,823,123, issued February 11, 1958; an alkali metal salt of a substituted amino acid such as disodium N-(carbo-p-tert. octylphenoxy-pentaethoxy)-glutamate as described in Knox and Wilson U.S. patent ap-

plication Serial No. 600,679, filed July 30, 1956; or a sulfo-succinamate such as tetrasodium N-(1,2-dicarboxyethyl)-N-octadecyl sulfosuccinamate or N-lauryl disodium sulfo-succinamate as described in Knox and Stenberg U.S. patent application Serial No. 691,125, filed October 21, 1957.

In the preparation of the silver halide dispersions employed for preparing silver halide emulsions, there may be employed as the dispersing agent for the silver halide in its preparation, gelatin or some other colloidal material such as colloidal albumin, a cellulose derivative, or a synthetic resin, for instance, a polyvinyl compound. Some colloids which may be used are polyvinyl alcohol or a hydrolyzed polyvinyl acetate as described in Lowe U.S. Patent 2,286,215, issued June 16, 1942; a far hydrolyzed cellulose ester such as cellulose acetate hydrolyzed to an acetyl content of 19-26% as described in U.S. Patent 2,327,808 of Lowe and Clark, issued August 24, 1943; a water-soluble ethanolamine cellulose acetate as described in Yutzy U.S. Patent 2,322,085, issued June 15, 1943; a polyacrylamide having a combined acrylamide content of 30-60% and a specific viscosity of 0.25-1.5 on an imidized polyacrylamide of like acrylamide content and viscosity as described in Lowe, Minsk and Kenyon U.S. Patent 2,541,474, issued February 13, 1951; zein as described in Lowe U.S. Patent 2,563,791, issued August 7, 1951; a vinyl alcohol polymer containing urethane carboxylic acid groups of the type described in Unruh and Smith U.S. Patent 2,768,154, issued October 23, 1956; or containing cyano-acetyl groups such as the vinyl alcohol-vinyl cyano-acetate copolymer as described in Unruh, Smith and Priest U.S. Patent 2,808,331, issued October 1, 1957; or a polymeric material which results from polymerizing a protein or a saturated acylated protein with a monomer having a vinyl group as described in U.S. Patent 2,852,382, of Illingsworth, Dann and Gates, issued September 16, 1958.

If desired, compatible mixtures of two or more of these colloids may be employed for dispersing the silver halide in its preparation. Combinations of these antifoggants, sensitizers, hardeners, etc., may be used.

The Lowry Red (Wratten No. 92) filter referred to above transmits only radiation beyond about 630 m $\mu$  (i.e., absorbs substantially all radiation less than about 630 m $\mu$ ).

The invention has been described in detail with particular reference to preferred embodiments thereof, but it will be understood that variations and modifications can be effected within the spirit and scope of the invention as described hereinabove and as defined in the appended claims.

What we claim is:

1. A photographic reversal color process for processing a photoexposed multi-layer photographic element comprising a support and a photographic silver halide emulsion sensitive to the blue region of the spectrum, a photographic silver halide emulsion spectrally sensitized to the green region of the spectrum and a photographic silver halide emulsion spectrally sensitized to the red region of the spectrum, comprising developing said photographic element in a photographic developer for producing at least one black-and-white negative image but no color image, subjecting said photographic element to at least one reversal re-exposure, contacting the silver halide emulsion layers of said photographic element with an aqueous solution consisting essentially of water and at least 0.25 gram per liter of a compound selected from the class represented by the following general formula:



75 wherein R represents a member selected from the class

consisting of a hydrogen atom and a lower alkyl group,  $R_1$  represents a member selected from the class consisting of a hydrogen atom, an aryl group and an arylene-thiazolyl group,  $D$  represents the non-metallic atoms necessary to complete an aromatic nucleus,  $X$  represents an acid radical and  $n$  represents a positive integer of from 1 to 26 when  $R_1$  represents a member selected from the class consisting of a hydrogen atom and an arylene-thiazolyl group, and  $n$  represents a positive integer of from 1 to 3 when  $R_1$  represents an aryl group, and developing a color image in said photographic element by development in a photographic developer for producing a colored image and a positive silver image, said color development being carried out while a color-coupling component is dispersed throughout said silver halide emulsion layers.

2. A photographic reversal color process for processing a photoexposed multi-layer photographic element comprising a support and at least one photographic silver halide emulsion layer sensitive to the blue region of the spectrum, at least one photographic silver halide emulsion spectrally sensitized to the green region of the spectrum and at least one photographic silver halide emulsion spectrally sensitized to the red region of the spectrum, comprising developing said photographic element in a photographic developer for producing only a black-and-white negative image, contacting said silver halide emulsion layers with an aqueous solution consisting essentially of water and at least 0.25 gram per liter of a compound selected from the class represented by the following general formula:



wherein  $R$  represents a member selected from the class consisting of a hydrogen atom and a lower alkyl group,  $R_1$  represents a member selected from the class consisting of a hydrogen atom, an aryl group and an arylene-thiazolyl group,  $D$  represents the non-metallic atoms necessary to complete an aromatic nucleus,  $X$  represents an acid radical and  $n$  represents a positive integer of from 1 to 26 when  $R_1$  represents a member selected from the class consisting of a hydrogen atom and an arylene-thiazolyl group, and  $n$  represents a positive integer of from 1 to 3 when  $R_1$  represents an aryl group, subjecting said photographic element to a reversal re-exposure and producing a color image in said photographic element by color development in a color developer, said color development being carried out while a color coupling component is dispersed throughout said silver halide emulsion layers.

3. A photographic reversal color process for processing a photoexposed multi-layer photographic element comprising a photographic silver halide emulsion sensitive to the blue region of the spectrum, a photographic silver halide emulsion spectrally sensitized to the green region of the spectrum and a photographic silver halide emulsion spectrally sensitized to the red region of the spectrum, comprising subjecting said photographic element to development in a photographic developer for producing only a black-and-white negative image, followed by separate reversal re-exposure and color development for each of said emulsions in a photographic color developer containing a color-forming compound capable of coupling with the oxidation products of said photographic color developer to produce a colored image complementary to the region of the spectrum to which each of said photographic silver halide emulsions is sensitive, the photographic silver halide emulsions of said photographic element being treated after negative development but before any color development with an aqueous solution

40  
45

consisting essentially of water and at least 0.25 gram per liter of a compound selected from the class represented by the following general formula:

5

10



wherein  $R$  represents a member selected from the class consisting of a hydrogen atom and a lower alkyl group,  $R_1$  represents a member selected from the class consisting of a hydrogen atom, an aryl group and an arylene-thiazolyl group,  $D$  represents the non-metallic atoms necessary to complete an aromatic nucleus,  $X$  represents an acid radical and  $n$  represents a positive integer of from 1 to 26 when  $R_1$  represents a member selected from the class consisting of a hydrogen atom and an arylene-thiazolyl group, and  $n$  represents a positive integer of from 1 to 3 when  $R_1$  represents an aryl group.

4. A photographic reversal color process for processing a photoexposed multi-layer photographic element comprising a photographic silver halide emulsion sensitive to the blue region of the spectrum, a photographic silver halide emulsion spectrally sensitized to the green region of the spectrum and a photographic silver halide emulsion spectrally sensitized to the red region of the spectrum, comprising subjecting said photographic element to development in a photographic developer for producing only a black-and-white negative image, followed by separate reversal re-exposure and color development for each of said emulsions in a photographic color developer containing a color-forming compound capable of coupling with the oxidation products of said photographic color developer to produce a colored image complementary to the region of the spectrum to which each of said photographic silver halide emulsions is sensitive, the photographic silver halide emulsions of said photographic element being treated after negative development but before any color development with an aqueous solution consisting essentially of water and at least 0.25 gram per liter of a compound selected from those represented by the following general formula:

50



wherein  $R$  represents a member selected from the class consisting of a hydrogen atom and a lower alkyl group,  $R_1$  represents an aryl group,  $D$  represents the non-metallic atoms necessary to complete an aromatic nucleus,  $X$  represents an acid radical and  $n$  represents a positive integer of from 1 to 3.

5. A photographic reversal color process for processing a photoexposed multi-layer photographic element comprising a photographic silver halide emulsion sensitive to the blue region of the spectrum, a photographic silver halide emulsion spectrally sensitized to the green region of the spectrum and a photographic silver halide emulsion spectrally sensitized to the red region of the spectrum, comprising subjecting said photographic element to development in a photographic developer for producing only a black-and-white negative image, followed by separate reversal re-exposure and color development for each of said emulsions in a photographic color developer containing a color-forming compound capable of coupling with the oxidation products of said photographic color developer to produce a colored image complementary to the region of the spectrum to which

70

75

each of said photographic silver halide emulsions is sensitive, the photographic silver halide emulsions of said photographic element being treated after negative development but before any color development with an aqueous solution consisting essentially of water and at least 0.25 gram per liter of a compound selected from those represented by the following general formula:



wherein R represents a member selected from the class consisting of a hydrogen atom and a lower alkyl group, R<sub>1</sub> represents a hydrogen atom, D represents the non-metallic atoms necessary to complete an aromatic nucleus, X represents an acid radical and n represents a positive integer of from 1 to 26.

6. A photographic reversal color process for processing a photoexposed multi-layer photographic element comprising a photographic silver halide emulsion sensitive to the blue region of the spectrum, a photographic silver halide emulsion spectrally sensitized to the green region of the spectrum and a photographic silver halide emulsion spectrally sensitized to the red region of the spectrum, comprising subjecting said photographic element to development in a photographic developer for producing only a black-and-white negative image, following by separate reversal re-exposure and color development for each of said emulsions in a photographic color developer containing a color-forming compound capable of coupling with the oxidation products of said photographic color developer to produce a colored image complementary to the region of the spectrum to which each of said photographic silver halide emulsions is sensitive, the photographic silver halide emulsions of said photographic element being treated after negative development but before any color development with an aqueous solution consisting essentially of water and at least 0.25 gram per liter of a compound selected from the class represented by the following general formula:



wherein R represents a member selected from the class consisting of a hydrogen atom and a lower alkyl group, D represents the non-metallic atoms necessary to complete an aromatic nucleus, X represents an acid radical, and m represents a positive integer of from 1 to 26.

7. A photographic reversal color process for processing a photoexposed multi-layer photographic element comprising a photographic silver halide emulsion substantially sensitive only to the blue region of the visible spectrum, a photographic silver halide emulsion spectrally sensitized to the green region of the visible spectrum and a photographic silver halide emulsion spectrally sensitized to the red region of the visible spectrum, comprising subjecting said photographic element to development in a photographic developer for producing only a black-and-white negative image, exposing the red sensitive emulsion of said photographic element to red radiation, developing said red sensitive silver halide emulsion in a color developer containing a color-forming compound capable of coupling with the oxidation products of the color developing agent of said photographic color developer to produce a cyan image, the photographic silver halide emulsion spectrally sensitized to the red region of the visible spectrum being treated after negative development but before any color development with an aqueous solution consisting essentially of water and at least 0.25 gram per liter of a compound selected from the class represented by the following general formula:

16  
ment but before any color development with an aqueous solution consisting essentially of water and at least 0.25 gram per liter of a compound selected from the class represented by the following general formula:



wherein R represents a member selected from the class consisting of a hydrogen atom and a lower alkyl group, R<sub>1</sub> represents an aryl group, D represents the non-metallic atoms necessary to complete an aromatic nucleus, X represents an acid radical and n represents a positive integer of from 1 to 3, said photographic element being washed with water after treatment in said aqueous solution, and after production of said cyan image in said red-sensitized silver halide emulsion layer, exposing said blue sensitive silver halide emulsion layer to blue light and developing said blue sensitive silver halide emulsion in a photographic color developer for producing a yellow image in said blue sensitive silver halide emulsion layer, fogging the unexposed silver halide in said green-sensitized silver halide emulsion layer and developing said green-sensitized silver halide emulsion layer in a photographic color developer for producing a magenta image, the color-forming compounds for producing the respective yellow and magenta images being incorporated in the respective color developers.

8. A photographic reversal color process for processing a photoexposed multi-layer photographic element comprising a photographic silver halide emulsion substantially sensitive only to the blue region of the visible spectrum, a photographic silver halide emulsion spectrally sensitized to the green region of the visible spectrum and a photographic silver halide emulsion spectrally sensitized to the red region of the visible spectrum, comprising subjecting said photographic element to development in a photographic developer for producing only a black-and-white negative image, exposing the red sensitive emulsion of said photographic element to red radiation, developing said red sensitive silver halide emulsion in a color developer containing a color-forming compound capable of coupling with the oxidation products of the color developing agent of said photographic color developer to produce a cyan image, the photographic silver halide emulsion spectrally sensitized to the red region of the visible spectrum being treated after negative development but before any color development with an aqueous solution consisting essentially of water and at least 0.25 gram per liter of a compound selected from the class represented by the following general formula:



wherein R represents a member selected from the class consisting of a hydrogen atom and a lower alkyl group, R<sub>1</sub> represents a hydrogen atom, D represents the non-metallic atoms necessary to complete an aromatic nucleus, X represents an acid radical and n represents a positive integer of from 1 to 26, said photographic element being washed with water after treatment in said aqueous solution, and after production of said cyan image in said red-sensitized silver halide emulsion layer, exposing said blue sensitive silver halide emulsion layer to blue light and developing said blue sensitive silver halide emulsion in a photographic color developer for producing a yellow

image in said blue sensitive silver halide emulsion layer, fogging the unexposed silver halide in said green-sensitized silver halide emulsion layer and developing said green sensitized silver halide emulsion layer in a photographic color developer for producing a magenta image, the color-forming compounds for producing the respective yellow and magenta images being incorporated in the respective color developers.

9. A photographic reversal color process for processing a photoexposed multi-layer photographic element comprising a photographic silver halide emulsion substantially sensitive only to the blue region of the visible spectrum, a photographic silver halide emulsion spectrally sensitized to the green region of the visible spectrum and a photographic silver halide emulsion spectrally sensitized to the red region of the visible spectrum, comprising subjecting said photographic element to development in a photographic developer for producing only a black-and-white negative image, exposing the red sensitive emulsion of said photographic element to red radiation, developing said red sensitive silver halide emulsion in a color developer containing a color-forming compound capable of coupling with the oxidation products of the color developing agent of said photographic color developer to produce a cyan image, the photographic silver halide emulsion spectrally sensitized to the red region of the visible spectrum being treated after negative development but before any color development with an aqueous solution consisting essentially of water and at least 0.25 gram per liter of a compound selected from the class represented by the following general formula



wherein R represents a member selected from the class consisting of a hydrogen atom and a lower alkyl group, D represents the non-metallic atoms necessary to complete an aromatic nucleus, X represents an acid radical and m represents a positive integer of from 1 to 26.

5 10. A process according to claim 9 wherein said aqueous solution contains decamethylene-bis-benzothiazolium perchlorate.

11. A process according to claim 8 wherein said aqueous solution contains 3-ethylbenzothiazolium-p-toluenesulfonate.

12. A process according to claim 9 wherein said aqueous solution contains 3-(2-benzothiazolylmethyl)-2-methylbenzothiazolium-p-toluenesulfonate.

15 13. A process according to claim 9 wherein said aqueous solution contains pentamethylene-bis-2-methylbenzothiazolium perchlorate.

14. A process according to claim 9 wherein said aqueous solution contains hexamethylene-bis-benzothiazolium 20 perchlorate.

#### References Cited in the file of this patent

#### UNITED STATES PATENTS

|              |                    |                |
|--------------|--------------------|----------------|
| 2,356,486    | Weissberger et al. | Aug. 22, 1944  |
| 2,376,141    | Henn et al.        | May 15, 1945   |
| 2,384,663    | Weissberger et al. | Sept. 11, 1945 |
| 2,648,604    | Welliver et al.    | Aug. 11, 1953  |
| 2,694,716    | Allen et al.       | Nov. 16, 1954  |
| 30 2,899,306 | Spath              | Aug. 11, 1959  |